

## UNITED STATES PATENT OFFICE

2,454,541

## POLYMERIC DETERGENTS

Louis H. Bock, Huntingdon Valley, and James L. Rainey, Abington, Pa., assignors to Rohm & Haas Company, Philadelphia, Pa., a corporation of Delaware

No Drawing. Application September 9, 1944,  
Serial No. 553,476

6 Claims. (Cl. 260—53)

1

This invention relates to surface-active or capillary-active agents. It relates to the preparation of materials which have high detergent action under a wide variety of conditions. More specifically, it relates to the preparation and use of polymeric, water-soluble detergents which have high molecular weights and contain within each molecule a multiplicity of hydrophobic and hydrophilic groups or portions so arranged and balanced as to become oriented at an interface.

It is generally recognized that surface-active agents, as, for example, alkali-metal soaps or quaternary ammonium compounds, exist in water in the form of micelles. While the exact nature of such micelles is not established, there is evidence that they are electrically charged aggregates of molecules. For example, when a sodium soap of a fatty acid is dispersed in water, it dissociates into positively charged sodium ions and into negatively charged micelles which are aggregates of soap molecules and some negative ions. Because the micelles carry a negative charge, this type of soap is known as an anion-active detergent. In contrast, detergents of the type of quaternary ammonium compounds yield positively charged micelles in aqueous solution and, hence, are known as cation-active soaps or agents. This conception of the formation of micelles is based on measurements of freezing points, vapor pressures, and electrical conductivities of aqueous dispersions of surface-active agents. It is further recognized that surface activity is related to the formation of such micelles and to the orientation of the micelles at an interface.

The individual molecules in colloidal micelles are held together only by physical forces or by weak secondary valences; and, as a result, the extent of micelle formation depends upon the prevailing conditions, and it is affected by such factors as the concentration of the surface-active agent, the presence of electrolytes, solvents, and other surface-active agents, and also upon the temperature. Thus, dilution of the solution, elevation of the temperature, or a change in the amount of any salts which may also be present in solution favor the reversion of micelles into simple molecules and/or ions with the formation of true solutions. As an example, synthetic detergents known heretofore have no value at very low concentrations or in very hot water because under these conditions the micellar structure reverts, the molecules then exist in true solution, and, as a result, detergency is lost. The necessity of using relatively high concentrations plus the higher cost of synthetic detergents combines

2

to make the use of such detergents uneconomical and often impractical. Furthermore, the materials are ineffective in many laundering operations wherein extremely hot water is used in order to accelerate the removal of soil.

The products of this invention differ from—and have advantages over—detergents known heretofore in that their effectiveness is not dependent upon the formation of loosely bound micelles. By the process of this invention, water-soluble macromolecules are synthesized in which all of the bonds between atoms are primary valence links and, hence, are strong and are not affected by such factors as concentration and temperature. Furthermore, the synthesized macromolecules contain balanced hydrophilic and hydrophobic groups so positioned in the macromolecule that orientation can and does occur readily at an interface.

The products of this invention may be made by condensing hydrocarbon-substituted phenols with formaldehyde to produce polymeric materials which are in fact macromolecules and then introducing into said macromolecules hydrophilic groups. The hydrophilic groups, which impart water solubility, may be ether-alcohol groups or esterified ether-alcohol groups and are introduced, for example, by the reaction of ethylene oxide or propylene oxide with the macromolecule. If desired, the terminal hydroxyl of said ether-alcohol group may be converted into a salt-forming ester group of a polybasic acid.

The resultant products may be considered to have three functional portions. Thus, they contain (a) as the hydrophobic portion, the hydrocarbon groups attached to the phenol nucleus; (b) as the hydrophilic portion, the modified or unmodified ether-alcohol groups, and (c) as the polymeric portion, the phenol nuclei joined by methylene bridges. The hydrocarbon groups attached to the phenol and the modified or unmodified ether-alcohol groups also attached to the phenol are so balanced as to assure water solubility and orientation at an interface. At the same time, the polymeric nature of the product assures such a high molecular weight that the product is in fact a macromolecule which imparts capillary- or surface-activity to a solution, as do micelles of ordinary soaps, but which is stable and is not dissociated as are the micelles of customary detergents under adverse conditions.

The above discussion is for purposes of theoretical explanation only, and it must be understood that the so-called three portions of the 56 macromolecule are not independent of each other

but are all combined in one large molecule which functions as a concerted whole.

The type of hydrocarbon group which is attached to the phenol nucleus may vary as to kind but in every case must contain at least four carbon atoms. In reality, substituting groups of at least eight carbon atoms are much preferred. Generally, it is preferred that the substituent hydrocarbon group be a straight or branched chain acyclic group, such as n-butyl, iso-butyl, tertiary butyl, amyl, tertiary amyl, n-octyl, di-iso-butyl, decyl, dodecyl, hexadecyl, octadecyl, and the like. Alternatively, phenols substituted with alicyclic groups may be used. These are typified by cyclohexyl phenol, methyl-cyclohexyl phenol, butyl-cyclohexyl phenol, and dicyclohexyl phenol. While aryl-substituted phenols, such as p-phenyl phenol and p-naphthyl phenol, may be employed they are less satisfactory than those listed above unless they in turn contain an alkyl group. Thus, p-tolyl phenol is much preferred over p-phenyl phenol. Furthermore, a preference is given to the para-substituted phenols over those substituted in the ortho position. It is understood that although it is preferable to employ individual phenols, mixtures of phenols, for example, p-tert.-amyl- and p-diisobutyl-phenols, may be employed.

The ratio of formaldehyde should be between 0.5 and 1.0 mol per mol of phenol. The formaldehyde may be used in the form of a solution, such as the formalin of commerce, or in a polymeric form such as paraformaldehyde. Also, though not preferred, it may be in a form such as a formal or hexamethylene tetramine which will yield formaldehyde under the conditions of reaction.

Ordinarily, the substituted phenol and formaldehyde are reacted by condensing together in the presence of an acidic or alkaline condensation catalyst until the products have become relatively viscous. Solvents may be employed. Acidic condensation catalysts are preferred because of the ease with which the condensation may be controlled. Elevated temperatures naturally accelerate the rate of reaction. Condensation of formaldehyde and substituted phenols such as are here involved do not proceed to the infusible stage and, accordingly, no limit need be imposed upon the degree of condensation. In practice, it is convenient to follow the extent of condensation by means of viscosity measurements and the condensation may be halted at an early stage at which the molecular weight is low and the product on the average has no more than three or four phenolic units per molecule, or it may be continued until each macromolecule contains many more units. The condensation products may range in physical properties from oils to brittle solids, depending upon the degree of condensation and the nature of the substituent hydrocarbon group on the phenol.

Hydrophilic or water-solubilizing groups may be introduced by condensing with the substituted phenol-formaldehyde macromolecule an alkylene oxide such as ethylene oxide, a propylene oxide such as trimethylene oxide or isopropylene oxide, or a butylene oxide such as isobutylene oxide. The condensation is preferably conducted in the presence of an alkaline catalyst such as the hydroxides of the alkali metals, although in some instances no catalyst is required. While the reaction may be carried on at lower temperatures and at atmospheric pressure in the presence of solvents, it is preferred to conduct it at tempera-

tures above 100° C. under superatmospheric pressure with or without solvents. More than one mol of alkylene oxide is employed and, in fact, it is preferred to use at least eight mols per mol of phenol condensed in macromolecule. The product, which is water soluble and has capillary-action properties, may be represented by the formula

10



15

In the formula, R' represents a hydrocarbon substituent of four or more carbon atoms, R represents an alkylene group from the class consisting of ethylene, propylene, and butylene groups, y is an integer having a value of 8 or above and preferably from 10 to 20, inclusive, and x is an integer greater than 1.

20

It must be understood that mixtures of the alkylene oxides, such as a mixture of ethylene and propylene oxides, may be employed, although it is preferred to use individual oxides.

25

Alternatively, detergents having the above general formula may be made from the sodium derivative of the phenol-formaldehyde condensate and a halohydrin of a polyglycol such as Cl(C<sub>2</sub>H<sub>4</sub>O)<sub>7</sub>C<sub>2</sub>H<sub>4</sub>OH, Br(C<sub>2</sub>H<sub>4</sub>O)<sub>10</sub>C<sub>2</sub>H<sub>4</sub>OH, or Cl(C<sub>3</sub>H<sub>7</sub>O)<sub>6</sub>C<sub>3</sub>H<sub>7</sub>OH.

30

The products are best described as surface-active polymeric products containing in their chemical structure hydrocarbon-substituted phenoxy polyalkoxy alcohol units in which units said hydrocarbon substituent contains at least four carbon atoms and said alcohol contains at least eight oxygen-linked alkylene groups from the class consisting of ethylene, propylene, and butylene groups, at least three of said units being joined in each molecule by means of methylene bridges. The product may be esterified or etherified or otherwise modified to produce detergents of unusual properties. Such modifications are

45

the subjects of other of our applications.

50

The following examples will serve to illustrate the preferred method of preparing the surface-active products of this invention.

55

**Example 1**

Step 1.—Into a three-necked flask equipped with thermometer, mechanical agitator, and reflux condenser was charged the following: 412 grams of *a,a,y,y*-tetramethylbutylphenol, 162 grams of a 37% aqueous solution of formaldehyde, and 27.6 grams of water. The mixture was agitated and heated to a temperature of 90° C. At this point, 246 grams of oxalic acid and 0.92 gram of Twitchell's reagent dissolved in ten grams of water were added. While being agitated, the reaction mixture was refluxed for six hours. Two hundred grams of water and 384 grams of toluene were added, and refluxing was continued for an hour. Agitation was stopped and the contents of the flask were removed to a separatory funnel. The aqueous and resinous layers were separated and the solvent was removed from the resinous layer by vacuum distillation. After the removal of the solvent, heating at a reduced pressure of 1.5 to 2.5 mm. and at a temperature of 245° to 250° C. was continued for four and one-half hours. The condensate then had a viscosity of 4.0 poises when measured as a 60% solution in toluene and, on cooling, solidified to a brittle mass.

Step 2.—A mixture of 118 parts of the product of Step 1, having hydroxyl number of 260, two parts of solid NaH, and 100 parts of toluene was heated to 125° to 150° C. in an autoclave. Ethylene oxide was added slowly over a period of two and one-half hours until 261 parts of ethylene oxide were absorbed. This corresponds to eleven mols of ethylene oxide per mol of phenol in the product of step 1. The toluene was then removed by steam distillation and the water by vacuum distillation at 100° C. The product was obtained as a viscous paste having a corrected hydroxyl number of 97. It was readily soluble in water and had marked detergent properties. Its formula may be represented by the following:



*Example 2*

Step 1.—An octadecyl phenol-formaldehyde condensate was prepared by heating a mixture of 346 parts (1.0 mol) of octadecylphenol, 81 parts (1.0 mol) of 37% formaldehyde, 18.8 parts of water, 1.23 parts of oxalic acid, and 0.46 part of Twitchell's reagent for seven hours under reflux. One hundred ninety-two parts of toluene and 150 parts of water were added, and refluxing was continued for one-half hour. The aqueous layer was withdrawn and the toluene layer concentrated by removal of toluene under reduced pressure. The residue was finally heated for five hours at 250° C. at a pressure of 1.5 mm. of mercury. The product was a soft, viscous material, insoluble in water and having a hydroxyl number of 144 and a viscosity of 1.0 poise when measured as a 60% solution in toluene.

Step 2.—One hundred eighty parts of octadecylphenol-formaldehyde condensate, corresponding to approximately 0.5 mol of octadecylphenol, was treated with 440 parts (10.0 mols) of ethylene oxide in the manner described in Example 1. The product, which contained about twenty oxyethylene groups per octadecylphenol residue, had a corrected hydroxyl value of 55, was soluble in water, and displayed detergent properties.

Although the above examples are directed to the use of ethylene oxide, it is understood that a propylene oxide or a butylene oxide may be employed in a similar manner. In order to impart a given degree of water-solubility, it is advisable to use a greater amount of the higher oxides than the amount of ethylene oxide required. Furthermore, as the entire length of the hydrophilic group is increased, the product ordinarily becomes more water-soluble. It is, therefore, advisable to increase the hydrophobic group proportionately. This can be done by increasing the size of the hydrocarbon substituent of the phenol, as represented by R' in the above general formula. In this way, a balance is maintained between the hydrophilic and hydrophobic portions of the macromolecule so that the product is water-soluble and at the same time capillary-active, in that it becomes oriented at an interface.

A lower limit of eight mols of alkylene oxide per mol of phenol has been indicated above together with a preferred ratio of ten to twenty mols of oxide per mol of phenol. It is to be understood that the upper limit of the ratio can be

considerably above twenty to one. In fact, detergents have been prepared in which the ratio was as high as sixty to one. In such cases, the length of the hydrophobic group was also increased in order to assure a balance between the hydrophilic or water-solubilizing portions and the hydrophobic or water-insolubilizing portions.

In the above examples, the ethylene oxide is slowly added to the heated solution of the phenolic condensate. Alternatively, all of the materials may be mixed at the outset and then reacted at an elevated temperature, provided that precautions are taken to dissipate the heat evolved during the reaction.

15 All of the products of this invention function as capillary-active or surface-active agents. As such, they become oriented at an interface, lower the surface tension of water, and cause more rapid wetting of surfaces such as the surfaces of fibers as measured by the standard Draves Sinking Test. Their outstanding property is their effectiveness as detergents. In this capacity, as measured by wash tests and laundering tests, they are outstanding and are far superior to soaps and synthetic detergents known heretofore.

20 As detergents the products described herein may be used in hard water or in water of high salt content. They may be employed under acidic or alkaline conditions. Their advantage over synthetic detergents resides in the fact that they are not micellar but are in fact macromolecules which do not revert as do micelles. Thus, they are excellent detergents at very low concentrations or at very high temperatures where former synthetic detergents failed.

25 They are uncommonly advantageous in the laundering of cotton fabrics and in the scouring of wool, sized, dyed, and printed fabrics in general. They may be used for preparing dispersions of oil in water or dispersions of polymerizable materials prior to the polymerization thereof. Also, they serve to break water-in-oil emulsions such as are encountered in oil-fields. And they have been found to be very satisfactory in the treatment of leather, in the dispersion of pigments, and as assistants in dyeing.

30 The products of this invention are particularly useful when used in conjunction with other capillary-active agents, including fatty acid soaps and synthetic detergents such as those shown in United States Patents 2,115,192 and 2,143,759. Such combinations have extraordinarily high degrees of wetting and detergent properties.

We claim:

35 1. Water-soluble, polymeric detergents formed by condensing by heating (a) one mol of a phenol having the formula



40 in which R is a saturated hydrocarbon substituent containing eight to eighteen carbon atoms, and (b) from 0.5 to 1.0 mol of formaldehyde, and then reacting therewith (c) from eight to sixty mols of an alkylene oxide from the class consisting of ethylene oxide, propylene oxide, and butylene oxide.

45 2. Water-soluble, polymeric detergents formed by condensing by heating (a) one mol of a phenol having the formula



50 in which R is a saturated hydrocarbon substituent containing eight to eighteen carbon atoms,

and (b) from 0.5 to 1.0 mol of formaldehyde, and then reacting therewith (c) from ten to twenty mols of an alkylene oxide from the class consisting of ethylene oxide, propylene oxide, and butylene oxide.

3. Water-soluble, polymeric detergents formed by condensing by heating (a) one mol of a phenol having the formula



in which R is a saturated hydrocarbon substituent containing eight to eighteen carbon atoms, and (b) from 0.5 to 1.0 mol of formaldehyde, and then reacting therewith (c) from eight to sixty mols of ethylene oxide.

4. Water-soluble, polymeric detergents formed by condensing by heating (a) one mol of a phenol having the formula



in which R is a saturated hydrocarbon substituent containing eight to eighteen carbon atoms, and (b) from 0.5 to 1.0 mol of formaldehyde, and then reacting therewith (c) from ten to twenty mols of ethylene oxide.

5. Water-soluble, surface-active, polymeric

detergents formed by condensing by heating (a) one mol of octyl phenol and (b) from 0.5 to 1.0 mol of formaldehyde and then reacting therewith (c) from 10 to 20 mols of ethylene oxide.

6. Water-soluble, surface-active, polymeric detergents formed by condensing by heating (a) one mol of octadecyl phenol and (b) from 0.5 to 1.0 mol of formaldehyde and then reacting therewith (c) from 10 to 20 mols of ethylene oxide.

LOUIS H. BOCK.  
JAMES L. RAINY.

#### REFERENCES CITED

15 The following references are of record in the file of this patent:

#### UNITED STATES PATENTS

| Number    | Name      | Date          |
|-----------|-----------|---------------|
| 1,917,250 | Harris    | July 11, 1933 |
| 1,917,257 | Harris    | July 11, 1933 |
| 2,046,318 | Brubaker  | July 7, 1936  |
| 2,060,410 | Balle     | Nov. 10, 1936 |
| 2,076,624 | De Groote | Apr. 13, 1937 |

#### OTHER REFERENCES

Clayton-Theory of Emulsions, published by Blakiston Co., Philadelphia, Pa., 4th ed. (1943), page 127.